

## UNITED STATES PATENT OFFICE

2,114,109

MAGNETIC ALLOYS WITH HIGH INITIAL  
PERMEABILITYKotaro Honda and Tamotsu Nishina, Sendai,  
JapanNo Drawing. Application June 5, 1935,  
Serial No. 25,155

8 Claims. (Cl. 75—128)

This invention relates to improvements in magnetic alloys with high initial permeability and more particularly to an alloy consisting mainly of iron, nickel, tin, and chromium, and has for its object to provide a magnetic alloy which has a very high initial permeability in weak magnetic field with less hysteresis loss and higher specific electric resistance and which is easy to manufacture and to be worked.

10 The inventors have succeeded in producing a magnetic alloy consisting of iron, nickel, chromium and tin at the properly selected proportions and the alloy of this invention possesses very high initial permeability in a weak magnetic field and 15 a small hysteresis loss and a comparatively high specific electric resistance and also has stable magnetic properties for temperature variation and mechanical shock.

The alloy of this invention contains 10 to 60% of iron, 40 to 90% of nickel, 0.1 to 5% of tin, less than 5% of chromium as the main ingredients. The alloy of this invention may also contain as sub-ingredients from trace to 2% of each of titanium and silicon, and from trace to 25 1.5% of manganese. Silicon acts as a reducing agent and manganese is effective to facilitate cold working of the alloy. The alloy of the present invention may be subjected to heat treatment such as annealing which may be carried out by heating the alloy to the temperature of 30 about 1100° C. and then slowly cooling at the rate of about three degrees per minute in order to develop the most desirable characteristics and no quenching is necessary. Heretofore known 35 magnetic materials necessitating quenching have usually shown considerable difference in the effect of heat treatment corresponding to the proportion of length and diameter of the material, but the alloy of this invention shows almost no difference in size of material.

40 As actual examples, the alloy of this invention containing 14.3% of iron, 81.2% of nickel, 0.2% of tin and 3.0% of chromium, having in addition thereto 0.8% of silicon and 0.5% of manganese shows the initial permeability of 13,500.

45 By adding a proper amount of titanium to the above mentioned elements the initial permeability can be increased further. As for example, the alloy containing 10.3% of iron, 83.5% of nickel, 0.2% of tin, 4.0% of chromium, 0.5% of silicon, 0.5% of manganese and 1.0% of titanium shows the initial permeability of 19,800 which is much higher than the first example.

50 The most important characteristics of the alloy of this invention are mainly developed by the

addition of tin to the nickel-iron alloy or chrome-nickel-iron alloy. Though the element tin has no reducing effect, yet it is found by many experiments that the addition of tin increases the initial permeability of the alloy considerably 5 under the annealed state. The addition of titanium further improves the initial permeability of the alloy.

As it is evident from the foregoing description the alloy of this invention consists mainly of 10 iron, nickel, chromium and tin as the main ingredients with or without titanium, silicon and manganese as sub-ingredients and the alloy shows a very high initial permeability and has no aging effect and shows no change in the magnetic properties by temperature variation and its heat treatment is very simple since it needs no quenching and the necessary properties can be developed by the annealing process only. Accordingly the alloy of this invention is very well 15 adapted for magnetic materials for telephone and telegraph purposes.

What we claim as new and desire to secure by Letters Patent of the United States, is:

1. A magnetic alloy comprising 14.3% iron, 25 81.2% nickel, 0.2% tin and 3% chromium and in addition thereto 0.8% silicon and 0.5% manganese, said alloy having an initial permeability of 13,500, all proportions being approximate.

2. A magnetic alloy comprising 10.3% iron, 30 83.5% nickel, 0.2% tin and 4% chromium and in addition thereto 0.5% silicon and 0.5% manganese; said alloy also containing as an auxiliary element 1% titanium and having an initial permeability of 19,800, all proportions being approximate.

3. A magnetic alloy containing iron in the order of 10.3 to 14.3%, nickel in the order of 83.5 to 81.2%, chromium in the order of 4 to 3%, silicon about .5 to .8%, manganese about 40 5 and tin about .2%, said alloy being characterized by an initial permeability of the order of 13,000 or more.

4. A magnetic alloy characterized by the addition of tin to improve its magnetic qualities and 45 consisting of 10 to 60% of iron, 90 to 40% of nickel, 0.1 to 5% of tin and 0 to 5% of chromium as the main ingredients and from trace to 2% each of titanium and silicon and from trace to 1.5% of manganese as the sub-ingredients.

5. A magnetic alloy characterized by the addition of tin to improve its magnetic qualities and consisting of as essential ingredients 10 to 60% of iron, 90 to 40% of nickel and .1 to 5% of tin, and less than 5% chromium, characterized by 50 55

high initial permeability in a weak magnetic field, and no aging effect.

6. A magnetic alloy according to claim 5 including as another ingredient titanium to the extent of not over 2%.

7. A magnetic alloy characterized by the addition of tin to improve its magnetic qualities and consisting of as essential ingredients 10 to 60% of iron, 90 to 40% of nickel, .1 to 5% of

tin, from a trace to 2% of titanium and from a trace to 5% of chromium.

8. A magnetic alloy according to claim 7 including as further ingredients from a trace to 2% of silicon as a reducing agent and from a trace to 1.5% of manganese to facilitate cold working of the alloy.

KOTARO HONDA.  
TAMOTSU NISHINA.